# EUROPEAN PATENT SPECIFICATION

(11) **EP 0 694 932 B1**
(45) Date of publication and mention of the grant of the patent: **26.02.2003**
(21) Application number: 95304759.4
(22) Date of filing: 07.07.1995
(51) Int. Cl.: H01F 17/00, H01F 27/29

(54) **Inductor device**
Drosselspuleanordnung
Dispositif d'inductance

(30) Priority: 29.07.1994 GB 9415316
(43) Date of publication of application: 31.01.1996
(73) Proprietor: Intarsia Corporation, Fremont, CA 94539 (US)
(72) Inventor: Pedder, David John, Long Compton, Warwickshire CV36 5LB (GB)
(74) Representative: Harding, Richard Patrick

(56) References cited:
- EP-A- 0 398 485
- EP-A- 0 551 735
- PATENT ABSTRACTS OF JAPAN vol. 018 no. 442 (E-1593) ,17 August 1994 & JP-A-06 140267 (KYOCERA CORP) 20 May 1994,
- PATENT ABSTRACTS OF JAPAN vol. 008 no. 036 (E-227) ,16 February 1984 & JP-A-58 196005 (TOUTSUU:KK) 15 November 1983,
- PATENT ABSTRACTS OF JAPAN vol. 012 no. 362 (E-663) ,28 September 1988 & JP-A-63 116410 (FUJIKURA LTD) 20 May 1988,

## Description

There is a growing requirement, in the construction of very compact, low cost radios and other rf communications circuits, for small, high performance and cost effective inductor components.

Surface mountable chip inductors have recently become available that measure 2 by 1.25mm in area (a standard surface mount format), and that offer inductance values up to some 20 nH, with self resonant frequencies of 1 to 2 GHz and quality factors that peak at about 80 at about 0.5 of the self resonant frequency. These inductors are lithographically defined and employ a copper metallisation for low resistance and high quality factor. Such components are available at typical costs of 60 cents each, with costs predicted to fall to 30 cents each as production volumes rise.

Very compact inductors may also be realised in an integrated form within the upper metallisation layers of a multichip module type D (MCM-D) substrate structure. Such inductors can provide inductance values between 1 and 100 nH within a 1mm square footprint (using single or multilayer spiral structures), with self resonant frequencies between 20GHz and 500 Mhz. Quality factor in these MCM-D inductors is determined by the inductor resistance at low frequencies, while the peak quality factor is related to the nature and dielectric structure of the substrate employed. High resistivity silicon substrates with inductors defined in an aluminiumm-polyimide structure can provide quality factors between about 5 and 20, depending upon the inductor structure and inductance value. The peak quality factor occurs at a frequency between 0.25 and 0.5 of the self resonant frequency. MCM-D inductors on sapphire or other good dielectric substrates can achieve quality factors up to 30, with the peak quality factor occurring at about 0.5 of the self resonant frequency. The effective cost of such inductors is directly related to the cost per unit area of the MCM-D technology, which is currently about 20 cents per square mm and will fall to 5 to 10 cents per square mm as production volumes rise.

Patent No. GB 2290171 describes the construction of small, accurate discrete inductors that are to be assembled by flip chip solder bonding. These discrete inductors employ a spiral inductor structure defined in a low resistance copper metallisation layer on the upper surface of a small dielectric chip. Metallic vias are included to make connections between the spiral structure on the upper surface and solder bond connections on the lower surface.

Patent No. GB 2290913 describes the use of a ferrite chip located over a spiral inductor defined in an MCM-D substrate to increase the specific inductance value or the quality factor of the inductor. The ferrite chip is aligned and supported over the inductor by flip chip solder bonding.

According to the present invention an inductor device for mounting on a multichip module, on a direct-chip-attach assembly, or on a surface mount assembly, the multichip module, direct-chip-attach assembly or surface mount assembly comprising a first substantially planar substrate of electrically insulating material, said first substrate having formed thereon a plurality of electrically connective structures, comprises a second substantially planar substrate of electrically insulating material having first and second opposite major surfaces, a spiral metallisation structure formed on the first major surface of said second substrate defining an inductive element and a plurality of solder bumps formed on said first major surface, at least two of said solder bumps being formed on said spiral metallisation structure for electrically connecting said spiral metallisation structure to respective ones of said electrically connective structures on said first substrate.

In a preferred embodiment, the inductor device comprises a trimmable metallisation layer formed on the second major surface of said second substrate.

An inductor device in accordance with the invention will now be described by way of example with reference to the accompanying drawing, which shows the device diagrammatically in cross-section.

Referring to the drawing the inductor device comprises a copper metallisation 1 in a planar spiral format (square, circular or polygonal) defined on the lower surface of a dielectric material, high resistivity semiconductor or ferrite chip 2 about 1mm square. Suitable dielectric materials include polycrystalline or single crystal alumina (sapphire), or fused quartz, while silicon of greater than 2k.ohm cm resistivity is a suitable high resistivity semiconductor material. Ferrite materials may be selected according to the required permittivity and frequency of operation.

The inductor terminations on the lower face of the chip 2 are provided with solder bump connections 3 to allow flip chip solder bond assembly to mating solder bump or other solderable structures on the MCM, direct chip attach or surface mount substrate 4. Additional solder bond connections (7) may be included as required for mechanical support. The use of the flip chip solder bonding technique ensures precise lateral alignment and vertical spacing of the inductor chip 2 from the underlying substrate 4.

Apertures are defined in any power or ground plane structures in the substrate in the area over which the flip chip inductor 1 is mounted in order to minimise any inductance reduction through image inductance effects and any reduction in self resonant frequency from additional capacitive loading.

Single or multilayer inductors may be defined in this inductor structure, the latter providing higher inductance values for the same chip area. The multilayer inductors are constructed using a multilayer metal-polyimide or similar dielectric structure. The uppermost of the planar spiral inductor metallisation layers may also be separated from direct contact with the chip material by a layer of a low dielectric constant material 5 such as an organic polymer. This low permittivity dielectric layer 5 may be employed to minimise the interturn capacitance when high dielectric constant substrate materials, such as ferrites, are employed.

A further metallisation layer 6 may be defined on the upper surface of the inductor chip 2 to allow laser trimming of the inductance of this structure. This layer 6 provides an image inductance that acts to reduce the primary inductance of the spiral inductor 1 on the lower chip face. The level of inductance reduction depends upon the separation of the image plane 6 from the inductor 1 and the permeability of the chip material. The local removal and/or patterning of this exposed and accessible image inductor layer, for example using a laser beam, can then be used to adjust the effective overall inductance of the flip chip inductor device. Suitable patterning structures include concentric square or circular ring patterns and spiral structures. Concentric ring structures provide image eddy currents that can further reduce the effective inductance in step wise manner according to the number, dimensions and location of the rings with respect to the turns of the primary inductor 1. The concentric ring structures may then be cut to interrupt the individual eddy currents to provide a step wise trimming action that increases the inducance. On the other hand, the effective inductance variation resulting from the use of the spiral trimming action is continuous. Trimming of such inductors may be used to tune oscillator, filter or resonator circuits. The upper surface metallisation may be earthed by means of through-chip and substrate vias if required. The separation of the upper metallisation layer from the inductor, the chip to inductor gap determined by the flip chip solder bond height and the relative permittivity of the chip dielectric material will also determine the additional capacitance of this structure and the influence on the inductor self resonant frequency. For this reason low permittivity materials such as fused quartz may be preferred as the chip material.

The inductor structure may be defined on one face of a suitable substrate wafer in the following manner. A thin metallic adhesion layer (for example using a reactive metal system such as chromium, titanium or nichrome) and a plating seed layer (usually a thin copper layer) are sputter deposited onto the surface in succession. These layers may be between 0.05 and 0.5 micrometres in thickness in a typical case. The adhesion layer provides a strong bond to the chip surface. The copper layer provides a comparable surface onto which to plate additional copper. A thick layer of a photoresist material is applied to this face of the wafer and patterned to define a spiral opening structure into which the copper metallisation that forms the inductor itself is then plated. The copper plating should be of the maximum thickness consistent with good control of the plated structure and small spacing between inductor turns (for lowest resistance at a given inductor pitch and hence maximum quality factor). The inductor geometry will be limited by the resolution and feature aspect ratios that can be defined in the resist, together with the properties of the plating solution (throwing power and plating efficiency). Materials exist that can allow at least 25 micrometre copper thicknesses at feature separations of as little as 10 micrometres. This should lead to inductor peak quality factors of at least 100 in inductors of millimetre dimensions. After electroplating the resist mask and the plating seed layer and adhesion layer are stripped by suitable solvent and etchant treatments from all surface areas apart from where the inductors are defined.

Multilayer inductors (for example 2 or 3 layer inductors that give about 4 or 9 fold greater inductance per unit area than single layer inductors) may be produced as an extension of the single layer inductor structure by plating copper layers separated by a suitable dielectric such as a compatible polyimide. The multilayer structures require the definition of vias through the interlayer dielectric material. These may be produced by a number of techniques, including dry etching. A polyimide material may also be employed to provide a low permittivity layer between the inductor spirals and the chip material.

The completed single or multilayer plated copper inductor structure is then coated with a suitable passivation (for example a layer of silicon nitride) or a metallic, non-solderable barrier layer material (for example chromium or titanium). If a nonconducting passivation layer is employed, then vias are opened in this layer at the locations where input and output connections are required.

An array of solder bump structures are then defined over the inductor input and output points on the patterned inductor spiral and in a number of other locations as required for mechanical location and support.

The solder bump structure requires a solderable metallisation layer to which the solder bump itself is wetted and which defines the area of the solder bump on the surrounding passivation layer or non-solderable barrier metallisation area. Chromium-copper or chromium-copper-gold multilayer metallisation structures are suitable for this solderable metallisation requirement. The first, chromium layer provides adhesion and an ohmic connection to the underlying copper or barrier metallisation surface, while an alloyed chromium-copper layer follows that provides solderability without layer dissolution (for multiple solder bump melting operations). The final copper or copper-plus-gold layers provide initial solderability, these metals dissolving into the solder on bump reflow and reprecipitating on cooling as intermetallic compounds of tin. The gold, if employed, allows the solderable layer to be exposed to the atmosphere without oxidation prior to solder deposition. Solderable metallisation layers of this type may be defined by sequential vapour deposition through an etched metal foil or similar physical masking structure.

The solder itself may be a tin-lead eutectic composition (63Sn-37Pb by wt.- melting point 183°C) for direct chip attach or surface mount applications, or may be a 95Pb-5Sn composition (melting point 310°C) for MCM-D applications. The solder may be applied by electrodeposition using a seed layer and photoresist masking scheme similar to that described for the plating of the copper inductor structure on the first face of the wafer. Alternatively a physical masking structure may be employed with a vapour deposition process similar to that described for the solderable metallisation deposition. The solder may be deposited as separate layers of lead and tin or as an alloy.

After deposition and patterning of the solderable metallisation and solder layers, the solder bumps are reflowed by heating to above the solder liquidus temperature under inert or reducing atmosphere conditions. Solder bump diameters between 50 and 125 micrometres are considered appropriate for the flip chip inductor structure. Bump heights between 30 and 100 micrometres are suitable, depending upon the application. Such bump geometries are also typical for flip chip solder bonded ICs for MCM and DCA applications. Solder bumps are defined over the input and output connections to the inductor and also distributed across the chip surface to provide mechanical support for the mounted flip chip inductor. A typical flip chip inductor would employ 5 or 6 solder bumps comprising central and corner or edge bumps 3 for inductor contacts, plus three or four additional corner bumps 7 for mechanical support. A preferred flip chip inductor size would be 0.5, 1.0, 1.15, 1.5 or 2.0 mm on a side, giving some consistency with the trend in discrete surface mount component sizes. A square format may be preferred for inductors for MCM use, whereas a rectangular format would suit direct-chip attach and surface mount applications.

As noted above, a further metallisation layer 6 may be defined on the upper surface of the inductor wafer to allow laser trimming of the diced and mounted inductor structure. This layer 6 may employ a variety of metallisation materials, including, for example, titanium, chromium or aluminium or some combination of such materials. No lithographic or other patterning of this layer is required at the wafer fabrication stage and indeed this layer may be deposited, for example by sputter deposition, prior to the processing of the inductor face. The optical reflectivity and electrical resistivity of this layer will determine the ease of laser trimming and the losses in the inductor image plane.

The use of a photolithographic patterning process to define the inductor geometry enables very accurate inductor dimensions and hence highly reproducible inductor values. The use of copper as the inductor metallisation provides minimal inductor series resistance and hence maximum quality factor.

## Claims

1. An inductor device for mounting on a multichip module, on a direct-chip-attach assembly, or on a surface mount assembly, the multichip module, direct-chip-attach assembly or surface mount assembly comprising a first substantially planar substrate (4) of electrically insulating material, said first substrate having formed thereon a plurality of electrically connective structures, **characterised by** the device comprising a second substantially planar substrate (2) of electrically insulating material having first and second opposite major surfaces, a spiral metallisation structure (1) formed on the first major surface of said second substrate (2) defining an inductive element, and a plurality of solder bumps (3) formed on said first major surface, at least two of said solder bumps being formed on said spiral metallisation structure (1) for electrically connecting said spiral metallisation structure to respective ones of said electrically connective structures on said first substrate (4).

2. An inductor device in accordance with claim 1 wherein a trimmable metallisation layer (6) is formed on the second major surface of said second substrate (2).

3. An inductor device in accordance with claim 1 wherein said spiral metallisation structure (1) is formed on a layer (5) of low permittivity material deposited on said second substrate.

4. An inductor device in accordance with claim 2 wherein said trimmable metallisation layer (6) is formed in a concentric ring pattern.

5. An inductor device in accordance with claim 2 wherein said trimmable metallisation layer (6) is formed in a spiral pattern.

6. An inductor device in accordance with claim 1 wherein at least part of said spiral metallisation structure (1) is coated with a non-solderable metallisation layer.

7. An inductor device in accordance with claim 1 wherein at least part of said spiral metallisation structure (1) is coated with a layer of electrically insulating material.

8. An inductor device in accordance with claim 1 wherein said second substrate (2) is of ferrite material.

## Patentansprüche

1. Drosselspulen-Einrichtung für eine Anbringung auf einem Multichip-Modul, auf einer Direkt-Chip-Befestigungs-Anordnung oder auf einer Oberflächenanbringungs-Anordnung, wobei das Multichip-Modul, die Direkt-Chip-Befestigungs-Anordnung oder die Oberflächenanbringungs-Anordnung umfasst: ein erstes im wesentlichen planares Substrat (4) aus einem elektrisch isolierenden Material, wobei das erste Substrat darauf eine Vielzahl von elektrisch verbindenden Strukturen aufweist, **dadurch gekennzeichnet, dass** die Einrichtung ein zweites im wesentlichen planares Substrat (2) aus einem elektrisch isolierenden Material, welches erste und zweite gegenüberliegende Hauptoberflächen aufweist, eine spiralförmige Metallisierungsstruktur (1), die auf der ersten Hauptoberfläche des zweiten Substrats (2) ein induktives Element definierend gebildet ist, und eine Vielzahl von Lötbumps (3), die auf der ersten Hauptoberfläche gebildet sind, wobei wenigstens zwei der Lötbumps auf der spiralförmigen Metallisierungsstruktur (1) zum elektrischen Verbinden der spiralförmigen Metallisierungsstruktur mit jeweiligen der elektrisch verbindenden Strukturen auf dem ersten Substrat (4) gebildet sind.

2. Drosselspulen-Einrichtung nach Anspruch 1, wobei eine trimmbare Metallisierungsschicht (6) auf der zweiten Hauptoberfläche des zweiten Substrats (2) gebildet ist.

3. Drosselspulen-Einrichtung nach Anspruch 1, wobei die spiralförmige Metallisierungsstruktur (1) auf einer Schicht (5) aus einem Material mit geringer Permitivität, aufgebracht auf dem zweiten Substrat, gebildet ist.

4. Drosselspulen-Einrichtung nach Anspruch 2, wobei die trimmbare Metallisierungsschicht (6) in einem konzentrischen Ringmuster gebildet ist.

5. Drosselspulen-Einrichtung nach Anspruch 2, wobei die trimmbare Metallisierungsschicht (6) in einem spiralförmigen Muster gebildet ist.

6. Drosselspulen-Einrichtung nach Anspruch 1, wobei wenigstens ein Teil der spiralförmigen Metallisierungsstruktur (1) mit einer nicht-lötbaren Metallisierungsschicht beschichtet ist.

7. Drosselspulen-Einrichtung nach Anspruch 1, wobei wenigstens ein Teil der spiralförmigen Metallisierungsstruktur (1) mit einer Schicht aus einem elektrisch isolierenden Material beschichtet ist.

8. Drosselspulen-Einrichtung nach Anspruch 1, wobei das zweite Substrat (2) ein Ferritmaterial ist.

## Revendications

1. Dispositif d'inducteur pour un montage sur un module à multiples puces ou multipuce, sur un assemblage à fixation de puce directe ou sur un assemblage à montage en surface, le module multipuce, l'assemblage à fixation de puce directe ou l'assemblage à montage en surface comprenant un premier substrat sensiblement plan (4) en un matériau électriquement isolant, ledit premier substrat comportant formées sur lui une pluralité de structures de connexion électrique, **caractérisé en ce que** le dispositif comprend un second substrat sensiblement plan (2) en un matériau électriquement isolant qui comporte des première et seconde surfaces principales opposées, une structure de métallisation en spirale (1) qui est formée sur la première surface principale dudit second substrat (2) en définissant un élément inducteur et une pluralité de bossements de soudure (3) qui sont formés sur ladite première surface principale, au moins deux desdits bossements de soudure étant formés sur ladite structure de métallisation en spirale (1) pour connecter électriquement ladite structure de métallisation en spirale à certaines respectives desdites structures de connexion électrique sur ledit premier substrat (4).

2. Dispositif d'inducteur selon la revendication 1, dans lequel une couche de métallisation rognable (6) est formée sur la seconde surface principale dudit second substrat (2).

3. Dispositif d'inducteur selon la revendication 1, dans lequel ladite structure de métallisation en spirale (1) est formée sur une couche (5) en un matériau de permittivité faible qui est déposée sur ledit second substrat.

4. Dispositif d'inducteur selon la revendication 2, dans lequel ladite couche de métallisation rognable (6) est formée selon un motif en anneaux concentriques.

5. Dispositif d'inducteur selon la revendication 2, dans lequel ladite couche de métallisation rognable (6) est formée selon un motif en spirale.

6. Dispositif d'inducteur selon la revendication 1, dans lequel au moins une partie de ladite structure de métallisation en spirale (1) est revêtue d'une couche de métallisation non soudable.

7. Dispositif d'inducteur selon la revendication 1, dans lequel au moins une partie de ladite structure de métallisation en spirale (1) est revêtue d'une couche en un matériau électriquement isolant.

8. Dispositif d'inducteur selon la revendication 1, dans lequel ledit second substrat (2) est en un matériau de ferrite.
